

## UNITED STATES PATENT OFFICE

2,027,095

## COATING COMPOSITION

Earl D. Flood and John A. Hannum, Cleveland Heights, Ohio, assignors to The Flood Company, Cleveland, Ohio, a corporation of Ohio

No Drawing. Application December 17, 1931,  
Serial No. 581,776

1 Claim. (Cl. 134—49)

In wood-finishing, it has been quite customary heretofore to employ oil-filters and stains. The liquid material is applied to the surface, usually by brushing, spraying, etc. This is then allowed to set and thicken by drying somewhat, and is then carefully but vigorously worked into the wood. After the working-in operation, the excess is rubbed off until the surface is satisfactorily smooth. The filler is allowed to dry and then the finishing coats of shellac, varnish, lacquer, enamel or whatever is employed, are applied. In such operations, with oil-type fillers, there has been an initial difficulty that if the filler be made up complete much in advance of the time of application, the suspended solids are prone to settle out and set to such an extent that it is almost impossible to re-suspend them for satisfactory use. For this reason, it has been usual to make up oil-filters in stiff or paste form, and then thin them down to applying consistency at the time they are to be used. This lack of a "ready-mixed" preparation has thus entailed considerable extra annoyance and uncertainty upon the user. A preparation eliminating all this nuisance would thus represent a real saving to the consumer, besides greatly facilitating his work. A preparation which, furthermore, provides highly favorable characteristics in application and in drying-time is accordingly desirable and of fundamental importance.

To the accomplishment of the foregoing and related ends, the present invention, then, comprises the features hereinafter fully described, and particularly pointed out in the claims, the following description setting forth certain illustrative embodiments of the invention, these being indicative however, of but a few of the various ways in which the principle of the invention may be employed.

In accordance with the present invention, we make up a composition including an aqueous solution and a filler of an expander or crystallizing binder-type, and occasionally a drying oil. One of the greatest difficulties heretofore with any filler is a tendency to shrinkage. This has been serious enough in an oil-filler, where practically no evaporation takes place, but it has been much more aggravated with a water-filler where practically all of the drying is by evaporation. In such a case, it follows that the material would shrink in volume as it lost moisture. Correspondingly, the pores are only partially filled when the material has dried. As indicated, with our invention this shrinkage tendency is counteracted,

even with the use of water, by filler combinations of expanding tendency or crystallizing binders. In the former there is involved one or more components which may be subject to some action or reaction with one or more components of a subsequent coat, and by the latter is meant a crystallization or other deposition of one or more components in such a manner that the resulting volume of the solid is greater than the volume of the liquid from which it was deposited. For example, a substance such as sodium salicylate will crystallize in long slender needles of relatively great tensile strength but relatively weak shear strength. Such a material crystallizing in wood-pores will grow readily into the center of the pore through the body of the filler material and firmly anchor it in place against shearing stresses across the top surface, the crystals being in a position within the pores oriented in line with the tensile-stress. The material on the surface however, is anchored by crystals which grow at right angles to the direction of wiping and are hence easily sheared across and offer little resistance to the wiping operation. Usage of sodium salicylate affords a further function of an antiseptic character, which is desirable in the event of inclusion of organic materials susceptible to the action of molds, bacteria, and the like. Organic colloids which may be included are pentosan-type colloids, rubber latex, and in some instances glue, starch, etc. In addition to the drying oil, turpentine and benzene as thinners may be employed. Triethanolamine as such, or reacted with a fatty acid material to form soaps, is also desirable in small proportion. Finely divided mineral material is also advantageously incorporated, such as finely ground quartz, silica, mica, etc.

Compositions in accordance with the present invention are particularly favorable for the inclusion of a stain. By reason of the presence of water, a water-soluble stain-component may be included, and a water-soluble dye is much more satisfactory than an oil-soluble dye in practice, oil-soluble dyes being usually fugitive or having a tendency to fade on exposure to light, and they usually also leave the surface with a muddy appearance rather than clear and brilliant. As water-soluble stains we may include aniline dye or natural dye stuffs, pigments, or pyrogallol or the like treated with an oxidizing agent, for instance potassium or sodium bichromate, in alkaline solution.

By way of illustration, the following examples may be noted:

## I

|                               |    |      |
|-------------------------------|----|------|
|                               |    |      |
| Quartz (400 mesh)             | 10 | gms. |
| Mica (160 mesh)               | 5  | gms. |
| Amorphous silica (silex)      | 5  | gms. |
| 5 White lead (ground)         | 10 | gms. |
| Oil mixture                   | 5  | cc.  |
| Rubber latex (commercial)     | 5  | cc.  |
| Wax emulsion                  | 10 | cc.  |
| Shellac emulsion              | 15 | cc.  |
| 10 Stain solution             | 15 | cc.  |
| Pentosan colloid (commercial) | 6  | gms. |
| Glue                          | 1  | gm.  |
| Triethanolamine               | 2  | cc.  |
| 15 Sodium carbonate           | 6  | gms. |
| Sodium benzoate               | .5 | gm.  |

## II

|                             |     |      |
|-----------------------------|-----|------|
|                             |     |      |
| Stain solution              | 80  | cc.  |
| Rubber latex                | 15  | cc.  |
| 20 Quartz (400 mesh)        | 25  | gms. |
| Pentosan colloid            | .14 | gm.  |
| Sodium carbonate            | .14 | gm.  |
| Sodium salicylate           | .5  | gm.  |
| 25 Cellulose acetate powder | 7.5 | gms. |
| Mica (160 mesh)             | 30  | gms. |
| Boiled linseed oil          | 7   | cc.  |
| Turpentine                  | 2   | cc.  |
| Benzene                     | 1   | cc.  |
| 30 Triethanolamine          | 1   | cc.  |
| Oleic acid                  | 1   | cc.  |

In such compositions, a filler may be had affording excellent properties in application and rubbing and drying, together with effective pore-holding of filler-material. And where staining-action additionally is desired, this may also be realized in an effective degree, particularly where water-soluble stains are employed, the combination permitting a highly uniform setting-in of the stain with the filler.

Other modes of applying the principle of the invention may be employed, change being made as regards the details described, provided the features stated in any of the following claims, or the equivalent of such, be employed.

We therefore particularly point out and distinctly claim as our invention:

A wood-filling composition, comprising an aqueous vehicle, a predominant proportion of finely-divided mineral filler, and small proportions respectively of cellulose acetate, rubber latex, a drying oil, and crystallizing sodium salicylate.

EARL D. FLOOD.  
JOHN A. HANNUM.